

J. F. MONNOT.

PROCESS OF PRODUCING COMPOUND METAL BODIES.

APPLICATION FILED NOV. 12, 1906.

910,564.

Patented Jan. 26, 1909.



WITNESSES:

*W. Hauserstein*  
*Harry Gross.*

INVENTOR

*John F. Monnot*

BY

*Marble & Melloy*  
ATTORNEYS

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## PROCESS OF PRODUCING COMPOUND METAL BODIES.

No. 910,584.

Specification of Letters Patent.

Patented Jan. 26, 1909.

Application filed November 12, 1906. Serial No. 343,033.

To all whom it may concern:

Be it known that I, JOHN F. MONNOT, a citizen of the United States, residing at New York, in the county of New York and State 5 of New York, have invented a certain new and useful Process of Producing Compound Metal Bodies; and I do hereby declare the following to be a full, clear, and exact description of the same, such as will enable 10 others skilled in the art to which it appertains to make and use the same.

My invention relates to a process of producing compound metal bodies composed of layers or strata of unlike metals welded together (such as iron or steel, autogenously and completely welded to copper, silver, gold, 15 brass, bronzes, aluminum, etc.).

My invention consists in the novel method of weld-uniting unlike metals such as described.

According to my said invention I place within a suitable mold, a sheet or layer of one of the said metals, preferably the one of lower melting point, and then pour into the 25 mold the other said metal, causing the molten metal to solidify against the surface of the first metal, and to unite therewith. After the ingot has solidified it is subjected to working to condense the cast metal and to 30 insure perfect union between the metals.

In uniting unlike metals by casting one against the other, as described, it is exceedingly important, in order that there may be perfect union at all points between the cast 35 metal and the metal against which the same is cast, that the surface of the latter metal subjected to the action of the molten metal, shall be entirely clean and free from oxid, scale, etc., and that it shall be maintained in 40 such condition during the operation. This perfect cleanliness of surface has been very difficult, if not impossible, to secure by the methods heretofore used. The solid metal, particularly if thin, is heated up rapidly by 45 the molten metal, as the latter rises in the mold, and the hot metal still exposed to air tends to oxidize very rapidly. Furthermore, steel as ordinarily cast, carries with it considerable quantities of oxygen and other 50 gases some of which tend, or may tend, to attack the surface of the copper or other metal against which the steel is cast, or to make blow-holes, pores, or flaws at the point of union of the two metals, which flaws or

the like persist during the subsequent working of the ingot.

According to my invention I secure and preserve a clean surface of the solid metal, and prevent oxidation or other attack thereof, by cleaning the said surface initially and 60 then keeping it clean, both by maintaining a non-oxidizing or protective atmosphere in the mold and by covering such surface with a protective coating of fusible deoxidizing material, or by either of said methods separately; though preferably both are used together, the coating of fusible, deoxidizing material serving to clean the surface of oxids as it fuses under the heat of the casting operation and the neutral atmosphere serving to 70 maintain the clean surface when once formed. For the non-oxidizing or protective atmosphere I may employ producer gas made from coke, charcoal or anthracite, and which therefore contains no material proportion of 75 decomposable hydrocarbons. The protective paint may contain a powder of one or more of the readily-fusible oxygen-absorbing metals having a reducing power sufficient to reduce the oxids of the metals to be united 80 and, preferably contains a metal of the aluminum group, such as aluminum itself, magnesium, cadmium, etc. This powdered metal is to be mixed with water glass (silicate of an alkali) or other suitable binder. I find 85 it exceedingly advisable to pour the mold from the bottom and to place pieces of purifying material, such as aluminum, magnesium, cadmium, titanium, etc. (that is to say, any of the metals or substances which 90 are known to have a purifying or cleaning action on the steel or other molten metal) in the runner during the pouring. Thereby oxygen and other deleterious gases in the molten metal are removed. As the molten 95 metal is cast and rises in the mold, the protective coating mentioned melts away and rises as a slag, together with any aluminum or other oxid formed, thus exposing a clean surface to the action of the molten metal. 100 The coating, in so dissipating, tends to prevent collection of gases in bubbles or the like at the point of union of the two metals. By pouring the mold from the bottom I avoid 105 the entraining of air by the down-flowing stream of metal at a point so near the surface of the metal against which the molten metal is cast that there is not sufficient op-

portunity for elimination of oxygen by the aluminum or other purifying substance before contact with the solid metal occurs. By having a neutral atmosphere in the mold, 5 danger of oxidation of the powdered metal in the paint is avoided.

In the accompanying drawing I illustrate diagrammatically and in vertical section, apparatus such as may be employed for 10 carrying out my said invention.

I have shown apparatus arranged for producing a solid ingot coated on all sides with coating metal. But it will be obvious that my invention is not limited to producing 15 compound ingots coated on all sides, or to the production of solid coated ingots or ingots coated on the outside.

In the said drawings, 1 designates an ordinary ingot mold, 2 a pouring table, 3 a 20 runner for such table, and 4 a passage leading from the runner 3 to the ingot mold and entering same at the bottom. I customarily line the runner and the said passage with refractory material 5, as shown. Within the 25 ingot mold I place a hollow shell 7 composed of the metal of which the coating is to be made (copper for example), said shell being protected (preferably) on the side against which the molten metal is to be cast, with a 30 layer 8 of fusible protective material, such for example as a paint composed of aluminum powder and silicate of soda. Likewise the ingot mold is provided with a cap 9 having a pipe 10 for introducing a protective 35 atmosphere, such as producer gas; the gas so introduced being introduced at low pressure, and filling the mold, passing thence through passage 4 into the runner 3 and thence outward; or it may be burned in the runner, 40 or at the mouth thereof. Because of the low pressure at which the gas is introduced, it will not prevent the passage of molten metal from the runner into the mold, but will be forced back by the molten metal, 45 keeping all portions of the shell 7 not covered with the molten metal in a non-oxidizing atmosphere and preventing useless oxidation of the powdered metal in the protective paint.

50 Before applying the protective layer to the coating metal or metal against which the molten metal is to be cast, I first clean thoroughly the surface against which the molten metal is to be cast, and then apply 55 said coating, which then tends to prevent oxidation of the surface to be protected, even before the protective atmosphere is introduced into the mold. This protective coating in melting exerts to some extent a 60 specific cleaning action of its own.

In pouring a mold, molten metal is poured into the runner 3 and caused to pass through passage 4 into the ingot mold 1, forcing back into pipe 10 the protective 65 atmosphere, rising in the mold and as it

does so melting off the protective coating 8 and contacting with a clean metallic surface of the shell 7, the protective coating as it is melted off rising as a slag. I introduce into the runner, at suitable times, pieces of 70 aluminum, magnesium, cadmium, titanium, or other oxygen-absorbing or gas-absorbing or purifying material, so as to free the molten metal from gases dissolved therein or carried thereby and so insure a good quality of cast 75 metal and remove any oxygen present. The ingot having been cast as described, and the molten metal having solidified, the ingot is removed from the mold, and is worked, either directly or after submission to a soaking heat, whereby the cast metal is condensed and absolute union of the two metals is assured. This working may be effected by passing the ingot between rolls, or by subjecting it to the action of a press or a hammer, or by forcing the ingot, while the cast metal is still in a pasty condition, through a contracted die-orifice, as set forth in the Letters Patent to Edouard Martin and myself No. 853,932 dated May 14th, 1907 or the 80 metal may be subjected to pressure during and after solidification and while still pasty, to which end I may move the mold with the ingot within it under a press and apply pressure to the contents of the mold by means of 85 such press. Pressure applied on any of these ways prevents the molten metal from shrinking away from the other metal during 90 or after solidification.

Preferably the metal cast as above described is metal having a melting point near or higher than the melting point of the solid metal to be united to the metal so cast. In such case the molten metal causes fusion or semi-fusion of the surfaces of the coating 100 metal with which it contacts. For example, in the production of steel-copper or steel-silver ingots, I prefer that the copper or silver shall be used in solid condition and the steel cast molten against them. But when preferred or necessary, the metal of lower melting point, may be the metal which is cast; in such case the molten metal being heated 105 preferably to the supermolten condition, described for example in U. S. Letters Patent 110 granted to me on May 14th, 1907, No. 853,716.

It is obvious that while preferably both the coating of fusible material and the protective material and the protective atmosphere are employed together, and that while said coating and protective atmosphere co-operate to insure proper cleanliness of the surface against which the molten metal is cast, yet under some conditions one or the 115 other of these two protections may be omitted and the other used alone, but by conjoint use of the reducing protective paint and the neutral atmosphere important advantages are gained. The neutral atmos- 120 125 130

phere at casting temperature while preventing oxidation does not ordinarily have much effect in reducing oxids already formed, so that in operating without the reducing paint

- 5 it is necessary to have the surface of the metal shell very clean from the beginning while in using the protective paint alone, if it be, as it customarily is, a relatively thin layer or film, there is much danger of the air 10 in the mold oxidizing its contained powdered metal as the shell heats up under the heat of the advancing molten metal.

What I claim is:—

1. The process of uniting metals, which 15 comprises applying to a substantially clean surface of a body of one metal a fusible protective and deoxidizing coating containing a reducing body capable of reducing the oxids of the metals to be treated, casting against such surface a body of molten metal, and by the heat of the molten metal fusing such protective coating and causing same to leave the coated surface thereby exposing a clean metallic surface to the action of the molten 25 metal.

2. The process of uniting metals, which comprises applying to a substantially clean surface of a body of one metal a fusible protective coating comprising a readily fusible 30 metal capable of reducing oxids of the metal of such body, casting against such surfaces a body of molten metal, and by the heat of the molten metal fusing such protective coating and causing same to leave the coated surface, 35 thereby exposing a clean metallic surface to the action of the molten metal.

3. The process of uniting metals, which 40 comprises applying to a substantially clean surface of a body of one metal a fusible protective coating comprising aluminum, casting against such surface a body of molten metal, and by the heat of the molten metal fusing such protective coating and causing same to leave the coated surface, thereby 45 exposing a clean metallic surface to the action of the molten metal.

4. The process of uniting metals, which 50 comprises applying to a substantially clean surface of a body of one metal a fusible protective coating comprising aluminum and a binder, casting against such surface a body of molten metal, and by the heat of the molten metal fusing such protective coating and causing same to leave the coated surface, 55 thereby exposing a clean metallic surface to the action of the molten metal.

5. The process of uniting metals, which 60 comprises applying to a substantially clean surface of a body of one metal a fusible protective coating comprising aluminum and silicate of an alkali, casting against such surface a body of molten metal, and by the heat of the molten metal fusing such protec-

tive coating and causing same to leave the coated surface, thereby exposing a clean 65 metallic surface to the action of the molten metal.

6. The process of uniting metals, which comprises applying to a substantially clean surface of a body of one metal a fusible protective coating comprising a gas-absorbing metal capable of reducing oxids of the metal coated, casting against such surface a body of molten metal and by the heat of the molten metal fusing such protective coating and 75 causing the same to leave the coated surface, thereby exposing a clean surface to the action of the molten metal.

7. The process of uniting metals, which 80 comprises applying to a substantially clean surface of a body of one metal a fusible protective coating comprising a metal of the aluminum group, casting against such surface a body of molten metal and by the heat of the molten metal fusing such protective 85 coating and causing the same to leave the coated surface, thereby exposing a clean surface to the action of the molten metal.

8. In uniting metals, the process which 90 comprises enveloping a surface of a body of one metal in place in a mold, with a protective non-oxidizing atmosphere, and introducing molten metal into said mold and thereby displacing such atmosphere and causing the molten metal to contact with 95 such surface.

9. The process of uniting metals, which 100 consists in enveloping a surface of a body of one metal in place in a mold, with a protective non-oxidizing atmosphere, said surface having applied to it a fusible protective coating, and introducing molten metal into said 105 mold and thereby displacing such atmosphere and melting and displacing the protective coating and causing the molten metal to contact with such surface.

10. The process of uniting metals, which 110 comprises placing a body of one metal within a suitable mold, protecting the surface of such body against chemical or other attack, by enveloping such surface with a displaceable substance, containing a reducing substance capable of reducing oxids of the metal of such body, purifying a body of molten metal by introducing therein a purifying substance 115 and then introducing such molten metal into the mold and causing same to displace such protective substance and contact with the surface protected.

In testimony whereof I affix my signature, 120 in the presence of two witnesses.

JOHN F. MONNOT.

Witnesses:

H. M. MARBLE,  
BYRON E. ELDRED.